

April 28, 1936.

E. C. DOMM

2,038,551

METHOD OF ELECTROPLATING ZINC ON CADMIUM ZINC ALLOYS

Filed Oct. 31, 1934



Trivator,  
Elgin Carleton Domm.  
By Dyringforth, Lee, Charlton & Willis.  
A. E. S.

## UNITED STATES PATENT OFFICE

2,038,551

METHOD OF ELECTROPLATING ZINC ON  
CADMIUM ZINC ALLOYSElgin Carleton Domm, Niles, Mich., assignor to  
National-Standard Company, Niles, Mich., a  
corporation of Michigan

Application October 31, 1934, Serial No. 750,875

8 Claims. (Cl. 91—70)

This invention relates to improvements in a method of coating metal.

This application is a continuation in part of my co-pending application Serial No. 653,549, filed January 25, 1933.

In the Crapo Patent No. 1,984,335, is described a method of coating a ferrous article by hot-galvanizing it with zinc, and over that depositing by some other method an additional coating of zinc.

It has now been discovered that in those methods the thickness of the undercoating may be decreased without injuring corrosion-resistance to the type of corrosion of which salt-spray is typical, if instead of the zinc undercoating an alloy of cadmium and zinc is used for such undercoating. At the same time, such an alloy may be applied at a lower temperature, and thus may be used in certain instances where the application of zinc alone by the hot-dip method might interfere with the character of the base.

The invention is particularly applicable to coating strands of wire to be used in reinforcing the bead of a tire. The wire when so used commonly acts as a tension-member, and is imbedded in a rubber or rubber compound. When so used, the wire is exposed to corrosive and rusting agents, particularly to moisture which may seep into the tire.

The drawing shows in diagrammatic form an embodiment of my invention.

In accordance with the invention, a metal, for example wire suitable for use in tire beads, is first hot-dipped to provide a coating of a cadmium-zinc alloy. This may be done, for example, by dipping the wire in a hot molten alloy of zinc and cadmium. Such an alloy always has a melting point lower than that of zinc, and certain of the alloys have a melting point below that of either zinc or cadmium.

A coating of zinc is then put over the first coat by electrolysis or electroplating. Not only does a double coating applied by the above mentioned method give very good corrosion-resistance, but it has been discovered that the electro-coat tends to fill in the depressions in the lower zinc-cadmium alloy coat and thus produce a uniform and smooth coating. A coating of the order of thickness of the lower coat is preferred.

If desired, copper or other suitable material may be applied over the corrosive-resistant double coating in order to increase the adhesiveness of the wire to rubber. It is frequently desirable to apply such a coating when wire is used as a reinforcement for a tire bead.

The new process herein described is especially useful in procuring a coating of a desired and uniform thickness. In practice, the wire is given

a hot coat first, and preferably I wipe this thin. In the next stage, the coating is put on by electroplating; the operation can be continued to give exactly a desired thickness. At the same time, the coating acquires a smooth, uniform character which is free from holes, defects, and the like.

As an example of the invention, it is preferred to use an alloy of approximately 80% zinc and 20% cadmium as the undercoating, because of its marked corrosion-resistance to the type of corrosion of which the salt spray is typical.

In general it is preferred that the alloy contain at least 10% cadmium and at least 30% of zinc.

The foregoing description has been given for clearness of understanding only, and no unnecessary limitations should be understood therefrom, but the appended claims should be construed as broadly as permissible in view of the prior art.

What I regard as new and desire to secure by Letters Patent is:

1. The process of coating a ferrous article which comprises applying to it by the hot-dip process a coating of an alloy of cadmium and zinc, and electrodepositing thereon an outer coating of zinc.

2. The method of coating a metal to increase its corrosion-resistance comprising first applying to it a molten zinc-cadmium alloy, and then applying a second coating of zinc over the first coating.

3. The method of producing a ferrous tire-bead reinforcement wire which comprises first coating a ferrous wire with a zinc-cadmium alloy by the hot-dip process, and then electroplating zinc over the hot-dipped wire to produce a uniform coating of desired thickness.

4. The method as set forth in claim 1, in which the zinc-cadmium alloy contains approximately 80 parts of zinc to 20 parts of cadmium.

5. A coated ferrous article, comprising a ferrous base having a hot-dipped coating of a zinc-cadmium alloy thereon, and over that an electrodeposited coating substantially wholly of zinc.

6. A coated ferrous wire comprising a ferrous base wire having a hot-dipped coating of a cadmium-zinc alloy thereon, and over that an electrodeposited coating substantially wholly of zinc.

7. A coated tire bead wire comprising a ferrous base wire having a hot-dipped coating of a zinc-cadmium alloy thereon, and electrodeposited coating substantially wholly of zinc thereon, and having a coating of rubber vulcanized thereto.

8. An article as set forth in claim 5, in which the zinc-cadmium alloy contains approximately 80 parts zinc to 20 parts cadmium.

ELGIN CARLETON DOMM.